

March 25, 1947.

J. N. DOW

2,417,916

METHOD OF MOTHPROOFING PILE FABRICS

Filed Oct. 31, 1941



Leavenworth  
James N. Dow

Richard W. Smith  
Attorney

Patented Mar. 25, 1947

2,417,916

# UNITED STATES PATENT OFFICE

2,417,916

## METHOD OF MOTHPROOFING PILE FABRICS

James N. Dow, Longmeadow, Mass., assignor to Bigelow-Sanford Carpet Co., Inc., Thompsonville, Conn., a corporation of Massachusetts

Application October 31, 1941, Serial No. 417,277

7 Claims. (Cl. 117—111)

1

This invention relates to the mothproofing of pile fabrics and its object is to provide an economical treatment for impregnating all of the pile yarn, including the tuft and base portions thereof, of a continuously advancing web of fabric with mothproofing agents of the substantive type which chemically combine with the wool molecule. My treatment is substantially uniform from end to end of the web.

The preferred embodiment of my invention includes the consecutive steps of impregnating the pile yarn with a substantive mothproofing agent in aqueous solution, steaming the impregnated fabric to effect exhaustion of the agent onto the pile yarn, followed by drying. As will be described, the liquor application is effected in such a way, preferably by pressing and wiping the solution into the pile, as to force the liquor into the base as well as the tuft portions of the pile yarn without causing any substantial absorption of the liquor by the threads of the backing fabric. Impregnation of the bases of the pile yarn is necessary for effective mothproofing, since the moth larvae tend to hide in the bases away from the light, yet by avoiding excessive impregnation of the backing threads I minimize waste, since those threads are of cellulosic material not attacked by moth larvae.

My method of application obviates any material exhaustion of mothproofing agent to the pile yarn until after the fabric leaves the liquor supply so that I insure maintenance of the liquor at a substantially unvarying concentration and I thereby insure that a long web of fabric receives a substantially unvarying amount of agent from end to end of the web.

By treating the pile yarn of a woven fabric, as contrasted with treating the raw wool stock, I effect substantial economies by avoiding the waste of expensive mothproofing chemicals as the result of lost raw stock fiber during the picking, carding, spinning, winding and weaving operations necessary to convert the raw stock into woven pile. As contrasted with mothproofing the spun yarn prior to weaving, I not only reduce waste but also obviate the loss of bloom or tuft flare in the finished fabric which would result from adhesion together of the tuft fibers when they are cut off during the weaving.

My treatment is therefore not only effective but inexpensive and I have achieved this result even in Jacquard fabrics where the base of the yarn is buried between upper and lower layers of cellulosic weft.

In the drawing:

Fig. 1 represents diagrammatically apparatus which may effectively be employed to carry out the treatment embodying my invention; and

Fig. 2 is a detail warpwise section of my novel mothproofed fabric.

The pile fabric 2, having pile 2a and a backing 2b, enters the machine around idlers 4 and 6,

2

being drawn in succession over a mothproofing liquor application device 10, through a steamer 12 and a drier 14. The fabric is advanced in the direction indicated by arrows by means of the rolls 16, 20 and 24, having respectively spikes 18, 22 and 26 protruding from their peripheries and adapted to engage and grip the backing 2b of the fabric. The spike rolls 16 and 20 are driven from a power source 30 whose speed can be varied to change the speed of advance of the fabric and which is connected by chain 32 to a sprocket 34 fixed to the shaft 36 to which roll 20 is secured. A chain 38 passes around sprocket 40 also secured to shaft 36 and around another sprocket 42 fixed to shaft 44, to which roll 16 is secured, to drive roll 16 from roll 20. Spike rolls 16 and 20 have the same peripheral speed. Spike roll 24 is driven from an independent variable speed power source 50 by means of chain 52 passing around sprocket 54 fixed to shaft 56 to which roll 24 is secured.

The applicator 10 consists of an application roll 60 immersed in a tank 62 containing mothproofing liquor 64 heated in any suitable manner, such as is indicated diagrammatically by the steam pipes 66. The application roll 60 is secured to a shaft 70 to which is fixed a sprocket 72 driven by chain 74 from a variable speed power source 16.

To press the pile 2a of the fabric against the application roll 60, the fabric passes around idlers 82 and 87 which are so positioned with relation to the uppermost portion of the periphery of the roll 60 as to cause the fabric to be deflected, as indicated, during its travel over the roll. To increase such pressure I provide a tension device 8 which consists of a roll having spikes 9 adapted to engage the fabric and mounted coaxially with a brake drum 11 having a brake band 13 secured at 15 to the frame of the machine and connected at 17 to the lever arm 19 pivoted at 21 and having a weight 23 which may be adjusted lengthwise of the lever arm to vary the drag on the fabric and thereby increase or decrease the pressure between the fabric and the periphery of the application roll 60.

The application roll 60 is preferably rotated, as indicated by the arrow, in a direction contrary to the direction of advance of the fabric.

After the fabric leaves the application roll its pile rubs over a presser bar 90, effective to press the liquor carried by the pile into the pile and effect better penetration.

The fabric, while its pile yarn is wet with the mothproofing liquor, immediately passes into steamer 12 filled with steam from a suitable source, as indicated by the steam pipes 100. The steamer may be of any desired construction provided it is of sufficient length to effect adequate steaming of the fabric as required to exhaust onto its pile yarn the mothproofing agent carried in solution by it. I have shown diagrammatically a festoon steamer with festoon rods 102 advanced in conventional manner to convey

the fabric through the steamer in hanging festoons, as indicated at 110. Upon emergence from the steamer, the fabric passes into a loop 112 and then is tensioned by the tension roll 120 having spikes engaging the fabric backing and a brake band 122 whose tension is made adjustable by the weighted lever 124 just as described above in connection with the tension roll 8.

From the tension roll 120 the fabric passes through drier 14 which may be of any desired construction and into which hot drying air is suitably admitted, as indicated by the conventional hot air inlet 130 and outlet 132. The length of the drier 14 should, of course, be sufficient to effect complete drying of the fabric before it emerges and passes around the drive cylinder 24 to the next succeeding step in the manufacture, as indicated at 150.

The liquor in tank 10 comprises a solution of a mothproofing agent of the type which is substantive to wool. I may use any of the known types of such agents but I prefer to employ pentachloro - dihydroxy - triphenyl-methane-sulphonate-acid of the nature available to the trade under the name "Eulan CN." Another suitable material is an organic silicofluoride of high molecular weight available as "Amuno." Still other suitable materials of the substantive type may be used. Taking Eulan CN as typical, I shall describe my invention with respect to its use.

The formula for a bath which I have used successfully in practice comprises 1 ounce Eulan CN per gallon of hot water (180° F.) to which is added .25% by weight, based on the combined weight of Eulan CN and water, of 56% acetic acid.

As the fabric 2 advances pile downwardly over the application roll 60 in the direction shown by arrows, the roll rotates in a reverse or clockwise direction. The pile tufts are wiped and somewhat flattened by the surface of the roll and the vigor of this wiping action is accentuated by the pressure of the fabric against the roll resulting from its deflection, as indicated, going over the roll and the drag exerted by the tension device 8. My experiments have shown that between approximately 1½ and 2% of Eulan CN to the weight of wool exhausted onto the pile yarn will effect good mothproofing if distributed substantially uniformly over the tuft and base portions thereof, and in practice I have employed approximately 1½%. The quantity of mothproofing liquor entrained by the yarn at the application roll, and so distributed, is sufficient at the concentration of 1 ounce mothproofing agent per gallon of hot water to effect, when subsequently steamed, the exhaustion of that required amount of agent onto the tufts.

To effect such entrainment requires not only that the fabric press firmly against the roll 60 but also that the fabric and roll rotate at the proper speeds with relation to the construction of fabric being processed. Thus, if the fabric to be treated consists, for example, of 12 foot wide carpeting weighing 2.63 pounds per square yard, of which 1.18 pounds per square yard represents pile yarn, and assuming that the carpet advances at a speed of 48 inches per minute so that 14.03 pounds of carpeting or 6.29 pounds of pile yarn per minute pass over the application roll, a reverse peripheral speed of advance of that roll of 1270 inches per minute will deposit on the yarn approximately 1.65 gallons of solution per minute which, when exhausted to the yarn, will increase its weight by about 1½% allowing for

slight absorption by the backing threads. These values may, of course, be varied considerably and, generally speaking, the faster the speed of rotation of the roll relative to a given speed of advance of the fabric the more solution will be entrained by the tufts, and the faster the fabric is advanced the greater must be the peripheral speed of the application roll to deposit a given amount of solution.

By so forcing the pile yarn to entrain a sufficient quantity of the solution to effect the mothproofing desired, I am able to remove the fabric from the supply of mothproofing liquor before any material exhaustion of the agent on the yarn takes place. Thereby I insure that the mothproofing liquor is not weakened materially during the mothproofing of a continuous web so that the quantity of agent exhausted to the pile yarn is substantially unvarying from end to end of the web.

Upon leaving the application roll 60 the fabric is wiped by the presser bar 90, which aids evenness of impregnation of the mothproofing liquor throughout the fibers of the pile yarn, including both tuft and base portions thereof.

While the pile yarn is still wet with the mothproofing liquor the fabric passes through the steamer 12 to exhaust the mothproofing agent onto the yarn, such exhaustion being enhanced by the elevated temperature resulting from the steam and by the acidity imparted to the liquor by the acetic acid. In practice I have found that subjecting the fabric to saturated steam at atmospheric pressure or slightly above for approximately 20 minutes will suffice to complete the exhaustion of the agent onto the wool yarn. The steamer must, of course, be of sufficient length to satisfy the necessary requirements as to steaming time relative to the speed of advance of the fabric.

After steaming, the fabric is immediately dried in the hot air drier 14 where all of the moisture is removed. I prefer to keep the fabric under tension in the drier to obviate shrinkage.

The completely dried fabric is then ready for the final steps in manufacture, such as finish shearing and backing sizing. As shown in Fig. 2, the fabric backing 2b may conventionally be constructed of wefts 206 and 208, stuffer warps 202 and chain warps 204. The pile yarn is composed of tufts 2a extending from the backing and bases 2b extending around the wefts 208. Both the tuft portions 2a and the bases 2b extending around the wefts 208 are thoroughly impregnated with exhausted mothproofing agent as indicated at 200a and 200b respectively. The drawing represents ideal conditions, and in practice there would inevitably be some mothproofing agent in the backing threads as a result of capillarity. But a feature of my invention which has contributed largely to its success is that a large portion of the mothproofing agent is concentrated in the base portions of the pile yarn where the larvae hide, and this result has been attained by me in practice even with Jacquard fabrics where the bases of the yarn extend between layers of backing weft.

My invention is, of course, not to be limited to the details above described except as required by the appended claims. Thus, other ways of applying the mothproofing agent may serve for some needs, such as by the use of an application roll rotating in the direction of advance of the fabric. However, I greatly prefer to employ the method above described because it effects the

base penetration required without excessive waste in the backing threads. Furthermore, the concentration of agent in the liquor may be increased above that which I have specified, employing for the purpose organic solvents such as alcohols, ketones, ethers, esters and glycol derivatives. But in practice I have found that a normal concentration such as that above described is entirely adequate.

I claim:

1. The method of applying a mothproofing liquor to a pile fabric to impregnate the pile in and through the base portions of said pile without substantial impregnation of the threads of the backing fabric, which comprises feeding the fabric continuously and in said feeding compressing the pile to form a flat layer of pile covering the threads of said backing fabric, squeezing restricted quantities of a solution of a substantive mothproofing agent into said layer of pile and close to the base portions of said pile, whereby said solution impregnates said base portions, restricting the quantity of solution so applied so that no substantial amount penetrates through said layer of pile to enter the threads of the backing fabric, steaming said fabric while wet with said solution to exhaust said agent onto said pile and drying said fabric.

2. The method of applying a mothproofing liquor to a pile fabric to impregnate the pile in and through the base portions of said pile without substantial impregnation of the threads of the backing fabric, which comprises feeding the fabric continuously and in said feeding flattening the pile to form a flat layer with the ends of the pile pointed in the direction opposite to the direction of the feed of the fabric, applying restricted quantities of a solution of a substantive mothproofing agent to said flat pile layer and close to the base portions of said pile whereby said solution impregnates said base portions, while restricting the quantity of solution so applied to such limited amounts that no substantial impregnation of the threads of the backing fabric takes place, steaming said fabric while wet with said solution to exhaust said agent onto said pile and drying said fabric.

3. The method of applying a mothproofing liquor to a pile fabric to impregnate the pile in and through the base portions of said pile without substantial impregnation of the threads of the backing fabric, which comprises feeding the fabric continuously and in said feeding compressing the pile to form a flat surface against an applicator roll, squeezing restricted quantities of a solution of a substantive mothproofing agent carried by said applicator roll into said flat surface and close to the base portions of said pile, whereby said solution impregnates said base portions, while restricting the quantity of solution so applied to such limited amounts that no substantial impregnation of the threads of the backing fabric takes place, steaming said fabric while wet with said solution to exhaust said agent onto said pile and drying said fabric.

4. The method of impregnating the pile only of a pile fabric, including the roots of the pile, with a mothproofing liquor which comprises continuously feeding the fabric, rolling down the pile and resiliently squeezing it to a flattened condition on the backing fabric and simultaneously applying the liquor to the flattened pile and absorbing substantially all of the applied liquor into said pile.

5. The method of impregnating the pile only

75

of a pile fabric, including the roots of the pile, with a mothproofing liquor which comprises continuously feeding the fabric, rolling down the pile and resiliently squeezing it to a flattened condition and simultaneously applying the liquor to the flattened pile in an amount approximately 1½% to 2% of the weight of the pile yarn whereby substantially all of the applied liquor is absorbed by said pile.

10 6. The method of applying a mothproofing liquor to a pile fabric to impregnate the pile in and through the base portions of said pile without substantial impregnation of the threads of the backing fabric, which comprises feeding the fabric continuously and in said feeding compressing the pile to form substantially a flat surface against an applicator, applying restricted quantities of a solution of a mothproofing agent carried by said applicator onto said flat surface and close to the base portions of said pile, whereby said solution impregnates said base portions, and regulating the quantity of mothproofing agent applied by said applicator in proportion to the compression of the pile as determined by the tension of the web and its rate of travel to insure application of a predetermined maximum quantity of mothproofing agent essential to saturation of the pile structure but insufficient to saturate the backing fabric.

30 7. The method of applying a mothproofing liquor to a travelling pile fabric to impregnate the pile in and through the base portions of said pile without substantial impregnation of the threads of the backing fabric, which comprises feeding the fabric continuously and in said feeding compressing the pile to form substantially a flat surface against an applicator roll, applying a solution of a mothproofing agent carried by said applicator roll onto said flat surface and close to the base portions of said pile, and regulating the speed of rotation of said roll and its direction of travel in proportion to the tension and relative speed of travel of the fabric to insure a constant rapid application of a predetermined quantity of mothproofing agent essential to saturation of the pile structure and its base but insufficient to permit saturation of the backing fabric.

JAMES N. DOW.

#### REFERENCES CITED

The following references are of record in the file of this patent:

#### UNITED STATES PATENTS

| Number    | Name     | Date          |
|-----------|----------|---------------|
| 2,234,666 | Bulford  | Mar. 11, 1941 |
| 2,184,147 | Lowe     | Dec. 19, 1939 |
| 1,771,341 | McCollum | July 22, 1930 |
| 676,375   | Whipple  | June 11, 1901 |
| 545,420   | Bamford  | Aug. 27, 1895 |
| 1,850,413 | Porte    | Mar. 22, 1932 |
| 2,163,104 | Salzberg | June 20, 1939 |
| 1,659,598 | Funk     | Feb. 21, 1928 |

#### FOREIGN PATENTS

| Number  | Country | Date          |
|---------|---------|---------------|
| 484,991 | British | 1936          |
| 477,196 | British | Dec. 23, 1937 |

#### OTHER REFERENCES

American Dyestuff Reporter, vol. XIV, No. 8, pages 322-323.

Textile Colorist, vol. 47, pages 229-231.

Chem. & Ind., Dec. 3, 1938, pages 1143-1146.